

# United States Patent Office

2,743,184

Patented Apr. 24, 1956

1

2,743,184

## PHOTOGRAPHIC ANTIPLUMMING AGENTS AND EMULSIONS CONTAINING THEM

William B. Kendall, Rochester, N. Y., assignor to Eastman Kodak Company, Rochester, N. Y., a corporation of New Jersey

No Drawing. Application May 3, 1954,  
Serial No. 427,373

3 Claims. (Cl. 95—7)

This invention relates to improvements in the production of photographic images, such as images on paper supports, prepared from silver halide emulsions. More particularly this invention relates to silver halide emulsions having associated therewith a novel antiplumming or antibronzing compound which prevents image degradation of an exposed silver halide emulsion during processing.

Silver halide emulsions after exposure often are subject to image degradation during processing, that is, during development, fixing, washing, toning, etc., and particularly when they encounter the moist heat to which they are subjected on drying as when prints are subjected to ferrotyping or hot glazing. This degradation of the image frequently manifests itself as "plumming" or "bronzing."

Heretofore, various compounds have been proposed for use with silver halide emulsions to overcome such pluming and bronzing effects.

An object of the present invention is to provide a novel method of producing photographic images of superior quality. Another object is to provide a method for preventing image degradation of an exposed silver halide emulsion during processing. Still another object is to prevent pluming or bronzing of photographic prints during a hot glazing process. Another object of the invention is to provide compounds suitable for use as antiplumming agents in silver halide emulsions. Other objects will appear hereinafter.

In accordance with the present invention I have found that endothiophenyl thiadiazoline thiol, and its potassium salt, are effective antiplumming agents when employed with silver halide photographic emulsions during processing of an exposed silver halide emulsion which term includes one or more of the operations of developing, fixing, washing and drying.

Potassium endothiophenyl thiadiazoline thiol may be prepared by the method described in J. Prakt. Chem., 60, 206 (1899).



Potassium ethyl xanthate was prepared by adding 30 g. of carbon bisulfide to a solution of 16 g. of potassium hydroxide in 50 ml. of ethanol. To the resulting slurry, a solution of 20 g. of freshly-distilled phenylhydrazine in 60 ml. of ethanol was added gradually. The mixture at first thinned out, and then set up again. It was heated with stirring, on the steam bath for four hours, then half of the solvent was distilled off, and the solution cooled in an ice bath. The white, crystalline potassium salt which separated was removed by filtration, washed with a little cold alcohol, and finally with ether.

The free endothiophenylthiadiazolinethiol may be prepared by treating the potassium salt thereof with hydrochloric acid.

In employing these compounds as antiplumming or

2

anti-bronzing agents either one of them, or a suitable mixture thereof, may be added preferably to the emulsion layer or layers. They are also effective if added to the developing solution, or to other layers carried on the sensitive emulsion support such as the backing layer or supercoat. Alternately the sensitive layer may be bathed in a solution of the agent after exposure but prior to development. These agents are employed preferably in amounts between 0.1 and 4.0 grams per mol of silver halide in the emulsion.

These two compounds are very effective an anti-plumming agents when employed in any of the ways herein described including bathing the developed image in a solution of the compound after fixation. A suitable bath for example in an aqueous solution containing 0.5 to 2.0 grams per liter of the compounds.

My invention is further illustrated in the following examples:

### Example 1

An emulsion was prepared in accordance with Example 1 of U. S. Patent 2,596,756. To separate portions of this emulsion were added quantities of a 1:500 aqueous solution of potassium endothiophenyl thiadiazoline thiol equivalent to 0, 0.5, 1.0 and 2.0 grams per mol of silver. These separate portions were then coated on separate sheets of glossy baryta coated single weight paper at a rate of 700 sq. ft. per mol of silver. Two samples of each coating were exposed through a step wedge, developed, fixed and washed. One set of prints was dried without heat and the other set was dried on a ferrotyping drum at 180 to 200° F. The reflection D-max values obtained are tabulated below:

|     | Cone. | Dried without heat | Dried with heat |
|-----|-------|--------------------|-----------------|
| 0   |       | 1.88               | 1.32            |
| 0.5 |       | 2.00               | 1.82            |
| 1.0 |       | 1.98               | 1.96            |
| 2.0 |       | 2.00               | 1.98            |

A second series of experiments was performed in the same manner as the first except that different levels of potassium endothiophenylthiadiazoline thiol were used. The reflection D-max values obtained are tabulated below:

|      | Cone. | Dried Without Heat | Dried with Heat |
|------|-------|--------------------|-----------------|
| 0    |       | 1.88               | 1.46            |
| 0.10 |       | 1.90               | 1.52            |
| 0.25 |       | 1.92               | 1.63            |
| 4.0  |       | 1.80               | 1.76            |

### Example 2

The free endothiophenylthiadiazolinethiol was found to be as strong an antiplumming agent as the potassium salt, as the following will illustrate.

An emulsion was prepared according to Example 1 of U. S. Patent 2,596,756. To portions of this emulsion were added quantities of a 1:200 solution of endothiophenylthiadiazoline thiol dissolved in equal parts of methanol and acetone, and equivalent to 0, 0.5 and 2.0 g./mol of silver. These emulsions were then coated on glossy baryta-coated single-weight paper at a rate of 650 ft.<sup>2</sup>/mol of silver. Two samples of each coating were exposed through a step wedge, developed, fixed and washed. One set of prints was dried without heat, and the other

set was dried on a ferrotypic drum at 180-200° F. The reflection D-max values obtained are tabulated below:

| Cone.    | D-Max<br>Dried<br>Without<br>Heat | Dried<br>With Heat |
|----------|-----------------------------------|--------------------|
| 0.....   | 1.88                              | 1.72               |
| 0.5..... | 1.90                              | 1.78               |
| 2.0..... | 1.86                              | 1.86               |

While in this specification I have described my invention mainly with reference to the use of these anti-plumming agents in developing solutions and anti-plumming baths, my invention is not limited to such treatments. When the term "processing" is mentioned in this specification, any treatment given to the photographic material after exposure and up to the production of the final washed image is included within its scope. This includes, in the case of prints, the final hot glazing treatment. Hence, although the agent is preferably added in the developing solutions, when not already present in the photographic material, it may be added in the fixing bath or prior to washing since sufficient of the compound will be adsorbed to the silver grains to give the desired anti-plumming effect during hot glazing of the print.

I claim:

1. The method of preventing image degradation of an exposed silver halide emulsion during drying which comprises performing at least one of the steps of developing,

fixing, washing and drying said emulsion in the presence of a compound having the formula:



2. A photographic silver halide emulsion containing from 0.1 and 4.0 grams per mol of silver halide of a compound having the formula:



3. A photographic element containing a silver halide emulsion and from 0.2 and 7.0 milligrams per square foot of a compound having the formula:



References Cited in the file of this patent

UNITED STATES PATENTS

2,353,754 Peterson ----- July 18, 1944

FOREIGN PATENTS

471,339 Canada ----- Feb. 6, 1951